

Patented Feb. 7, 1928.

1,638,167

## UNITED STATES PATENT OFFICE.

KARL BERNHOEFT, OF OBERSCHEIDEN, GERMANY, ASSIGNEE TO GENERAL ELECTRIC COMPANY, A CORPORATION OF NEW YORK.

### METAL COMPOSITION.

No Drawing. Application filed January 7, 1927, Serial No. 159,745, and in Germany March 19, 1926.

The present invention relates to metal compositions consisting largely of aluminum and more particularly to such compositions which are adapted for use as electrical conductors.

While it is well known that the strength of aluminum may be increased by alloying it with certain metals, the addition of such metals, as a rule, lowers the conductivity of the aluminum. In my copending application Serial No. 130,359, filed August 19, 1926, of which the present application is a continuation in part, there is disclosed an alloy consisting of aluminum and cadmium, the cadmium content of the alloy varying from about .05 per cent to 3 per cent. The cadmium is added to molten aluminum and within the limit specified provides very uniform and satisfactory results. The cadmium acts as a purifier and contrary to all expectations increases the tensile strength of the aluminum without appreciably affecting its conductivity.

According to the present invention, I have found that it is possible to further improve certain physical properties of the aluminum-cadmium alloy described in my prior application by the addition of a small quantity of copper, iron or silicon. The addition of approximately .1 to 1 per cent of copper, iron or silicon to the alloy described in my prior application renders it more responsive to heat treatment and increases the tensile strength of the alloy about 2½ kilograms per square millimeter. The addition of these metals also has the effect of increasing the flexibility or bending coeffi-

cient of the alloy by about 40 per cent. Although the present alloy has a tensile strength which is approximately 50 per cent greater than that of pure aluminum, the conductivity of the alloy is not noticeably less than the conductivity of pure aluminum, thus rendering the alloy particularly adaptable for use as an electrical transmission conductor.

Although I have claimed the element copper as a part of the combination in certain of the following claims, I do not intend that such claims should be limited to the use of copper, as it will be understood that either iron or silicon is the full equivalent of copper and may be used in its place if desired.

What I claim as new and desire to secure by Letters Patent of the United States, is—

1. A metal composition containing about .1 to 1 per cent of copper, .05 to about 3 per cent of cadmium and the remainder aluminum.

2. An electrical conductor consisting largely of aluminum and containing about .1 to 1 per cent of copper and about .05 to 3 per cent cadmium.

3. An alloy consisting largely of aluminum and containing about .05 to 3 per cent of cadmium and about .1 to 1 per cent of an other element, said alloy having an electrical conductivity substantially equal to that of pure aluminum and a tensile strength greater than that of pure aluminum.

In witness whereof, I have hereunto set my hand this 17th day of December, 1926.

KARL BERNHOEFT.